

Feb. 9, 1926.

1,572,461

R. A. BEAUSEJOUR

APPLICATION OF CELLULOSE ESTER LACQUERS

Filed August 19, 1925

Fig. 1



Fig. 2



INVENTOR

Rene A. Beausejour.

BY

Pennell, Davis, Marvin and Edmunds

ATTORNEYS

## UNITED STATES PATENT OFFICE.

REME A. BEAUSEJOUR, OF PORT RICHMOND, NEW YORK, ASSIGNOR TO STANDARD VARNISH WORKS, OF NEW YORK, N. Y., A CORPORATION OF NEW YORK.

## APPLICATION OF CELLULOSE-ESTER LACQUERS.

Application filed August 19, 1925. Serial No. 51,201.

*To all whom it may concern:*

Be it known that I, REME A. BEAUSEJOUR, a subject of the King of Great Britain, residing at Port Richmond, in the county of 5 Richmond, State of New York, have invented certain new and useful Improvements in the Application of Cellulose-Ester Lacquers; and I do hereby declare the following to be a full, clear, and exact description 10 of the invention, such as will enable others skilled in the art to which it appertains to make and use the same.

My invention relates to improvements in the application of cellulose ester lacquers. 15 The lacquers to which I particularly refer comprise a solution of a cellulose ester, such as cellulose nitrate or cellulose acetate, in a solvent or mixture of solvents, such as ethyl acetate or butyl acetate or a mixture of the 20 two. Such lacquers also usually include diluents such as toluol, turpentine or petroleum benzine, and may also include pigments as well as gums, such as ester gum, and plasticizers, such as castor oil or tricresyl 25 phosphate, for imparting special properties to the lacquer.

Such lacquers have been applied by various methods, such as brushing, flowing, spraying or dipping, but for the application 30 of such lacquers on a large scale to objects having considerable surface area, spraying is at present the most important method. These lacquers are hardened by the evaporation of their solvent or diluent content 35 and are comparatively quick-drying. For this reason it is difficult directly to obtain a smooth coating or a glossy coating, necessitating the use of a smoothing or polishing operation as part of the application of the 40 lacquer. The cellulose ester content of the lacquers, moreover, tends to be again softened on further contact with solvents therefor so that these difficulties are not avoided by the apparent expedient of applying successive coats. With spray application particularly, the resulting coat has a rough or 45 finely-pebbled surface.

In the application of lacquers to objects 50 having considerable surface area it accordingly has been necessary to employ smoothing or polishing operations, and, due to the character of the dried lacquer coats, particularly where deposited in a rough or uneven condition, these smoothing and polishing operations have involved considerable

time and labor and have been a large part of the expense of procuring a satisfactory finished coating, while at the same time over-intensive smoothing or polishing frequently resulted in marring of the finished surface, 60 leaving it deficient in finish or gloss and lustre.

More satisfactory results have been secured in lacquering small objects of a size such that they could conveniently be dipped without requiring excessive volumes of lacquer, but for practical purposes it is usually desirable to carry out the dipping operation upon a large number of such small objects at the same time. For the treatment either of a 70 large number of small objects or of objects having considerable surface area, a dipping bath of comparatively large volume has been required and this involves further difficulties. The lacquer compositions usually 75 employed are very inflammable and the fire risk is considerably increased. Evaporation losses are also much greater and the difficulties of maintaining the lacquer composition in the dipping bath constant are also 80 accentuated. Moreover, from the practical standpoint, the expense incident to the maintenance of a lacquer bath of large volume is not to be overlooked.

There have been proposals to apply certain types of coating compositions by dipping the objects to be coated through a relatively thin layer of the coating composition floating on an aqueous bath. Hitherto, however, the substantial exclusion of water 90 in any form from all operations which involve the use of cellulose ester lacquers has been considered essential, probably due to the blooming or blushing of the finish which always seems to accompany the presence of 95 water or moisture or water-vapor during the application of the lacquer to the object to be coated. Apparently, this predisposition of the art to avoid the presence of water in any form has discouraged any attempts to apply cellulose ester lacquers by such methods, but I have found that, by proper regard for the conditions of the operation, cellulose ester lacquers can be applied by an operation of this general type 100 with several important advantages.

In spite of the general experience of the art that the presence of water in any form must be avoided during the application of cellulose ester lacquers, I have successful- 110

ly accomplished the application of cellulose ester lacquers to both wooden and metallic objects from a layer of the lacquer floating on an aqueous liquid body, and I have secured improved results with respect to the character of the applied coating and unexpected results with respect to freedom of the applied coating from bloom or blush.

10 In carrying out my invention, I float a layer of the cellulose ester lacquer on an aqueous liquid body and I regulate the composition of the lacquer and of the liquid body so that the liquid body is substantially immiscible with the lacquer and, advantageously, so that the lacquer is substantially free from components which are soluble in or which dissolve water to any material extent. I then dip the object to 20 which the lacquer is to be applied through the floating layer of cellulose ester lacquer.

Some of the components of the lacquer may be more or less extracted by the aqueous liquid body without seriously interfering with the operation, but I find it best to correlate the composition of the liquid body and of the lacquer employed in any single operation so that the liquid body is substantially immiscible with the lacquer.

30 To accomplish these results, I may employ a saline liquid body of a composition such that it is substantially immiscible with the lacquer, or I may employ a lacquer composition substantially free from components 35 which are soluble in or which dissolve water, or I may employ such a liquid body in conjunction with such a lacquer composition.

Specific limitations of the composition 40 of the liquid body or of the composition of the lacquer cannot be given because they are mutually interrelated, and in any case the composition of the one to be employed will be somewhat dependent upon the composition of the other. For example, the saline solution employed may be a solution of sodium chloride, sodium sulphate, potassium chloride, potassium iodide, potassium sulphate, magnesium chloride, magnesium sulphate or calcium chloride. In general, I have found it advantageous to employ heavy solutions, such as saturated solutions or solutions of salts forming solutions of relatively high density, but it will be 55 apparent, for example, that with specific lacquer compositions certain salts may give better results than others. As a further example, with lacquer compositions substantially free from components which dissolve or which are soluble in water, water alone may be employed as the aqueous liquid body, whereas with a lacquer containing, for example, substantial amounts of ethyl alcohol better results are secured 60 by employing a saturated solution of

sodium chloride or potassium iodide as this decreases the miscibility of the aqueous body with the lacquer composition.

Commercial cellulose nitrate is usually transported and handled wet with ethyl alcohol to reduce the fire hazard, and the solvents and diluents employed in making up lacquers as commercially available frequently contain ethyl alcohol. This water-soluble and water-dissolving content of 75 lacquers made from these materials as commercially available are not to be disregarded if they are employed as such. According to my invention, however, I take care of such components as are introduced 80 into the lacquer compositions from such sources by correspondingly regulating the composition of the liquid body on which the lacquer layer is floated. In the case of ethyl alcohol, for example, I employ as a liquid body a water solution substantially saturated with, for example, sodium chloride or potassium iodide. The alcohol may also to some extent dissolve in the aqueous body but any such tendency may be counteracted by the addition of an appropriate amount of some other diluent immiscible with water or if the amount of alcohol so removed does not materially affect the 90 character of the lacquer, for example with respect to viscosity, this removal of alcohol may be ignored. Solvents and diluents and cellulose esters substantially free from such components may, however, be employed 95 with advantage. To reduce the fire hazard in handling cellulose nitrate, it may be wet with toluol instead of ethyl alcohol.

The accompanying drawings illustrate in a diagrammatic and conventional manner 105 apparatus adapted for carrying out my invention, and I will further describe my invention in connection therewith, but it will be understood that my invention can be carried out in other and different apparatus. In the accompanying drawings,

Fig. 1 represents in elevation and partly in section with parts broken away an apparatus adapted for carrying out my invention, and

Fig. 2 schematically illustrates, in a view corresponding to a transverse section through the dipping tank illustrated in Fig. 1, the 110 operation of my invention.

The drawings are not intended to be to scale, and in Fig. 2 particularly the film of lacquer on the panel undergoing immersion is shown in exaggerated form to adapt it to pictorial representation.

Referring to Fig. 1, a dipping tank 3 adapted to contain a liquid body 4 and a layer of lacquer 5 floating thereon is arranged beneath a vertically movable frame or track 6. The objects to be dipped are supported from a truck or carriage 7 which during the dipping operation is carried on

- the frame 6. The carriage 7 is movable on to and off of the frame 6 and by providing a number of these carriages successive dipping operations can be carried out rapidly by
- 5 running the carriage supporting the object or objects which have just been dipped off on the track and replacing it with a carriage supporting the object or objects next to be dipped. To provide for regular and
- 10 controlled vertical movement of the frame or track 6, one end of the frame is supported by a plunger 8 of a hydraulic jack 9 and the other end of the frame or track is supported by a wire rope or equalizing
- 15 cable 10 running over suitable pulleys and connected to the end of the frame or track adjacent the plunger so that vertical movement of the frame or track will be uniform at both ends. To operate the hydraulic
- 20 jack, fluid under pressure from connection 11 is supplied to the two-way valve 12 which also communicates with the chamber of the jack through connection 13 and an outlet connection 14. The valve 12 is ar-
- 25 ranged to permit the introduction of fluid under pressure from connection 11 into the jack chamber or to permit the escape of fluid from the jack chamber through connection 14 or to close the jack chamber. The valves
- 30 15 and 16 are provided in the fluid inlet and outlet connections respectively for regulating the rate of flow of fluid therethrough, and thereby, the rate of vertical movement of the track or frame 6.
- 35 Dipping apparatus of the type illustrated provides for uniform and regular motion of the object or objects to be dipped during the dipping operation and also enables the rate of motion of the object or objects
- 40 to be dipped both up and down to be closely controlled. I have found apparatus of this type to be advantageous in carrying out the invention, but it will be apparent that other dipping apparatus might be used.
- 45 In operation, the dipping tank 3 is partially filled with a liquid body of greater density than the lacquer composition to be employed and substantially immiscible therewith, and a layer of the cellulose ester lacquer is floated on this liquid body. The
- 50 amount of lacquer in the floating layer should be sufficient to supply the lacquer necessary to coat the objects to be dipped at least for a single operation and to insure the provision of a continuous film of lacquer about the objects to be dipped during immersion. The lacquer layer may, for example, be of a thickness of from something less than  $1\frac{1}{2}$ " up to 2 to 3" or more.
- 55 With a lacquer composition substantially free from water-soluble or water-dissolving components, water may be employed as the liquid body for floating the lacquer layer unless, due to the use of heavy pigments,
- 60 the density of the lacquer is greater than that of water. For floating heavier lacquers, or to promote the immiscibility of the aqueous body with the lacquer, a saline solution such as a solution of sodium chloride or potassium iodide may be used as
- 65 the liquid body. The object or objects to be dipped are then slowly immersed through the floating layer of lacquer until coated over so much of their surface as may be desired and are then withdrawn, the speed
- 70 of immersion and withdrawal being regulated to avoid undue disturbance of the floating lacquer layer and to allow for draining of excess lacquer from the coated object or objects.
- 75 The mechanism of the dipping operation itself will be clear from Fig. 2, and it may be directly observed by carrying out the dipping operation within a glass container.
- 80 As the object to be dipped, illustrated in the drawings as a wood panel 17, enters the dipping bath it first contacts with the floating lacquer layer so that a film of the lacquer is formed across its lower edge and as it continues to move downwardly through the floating lacquer layer a lacquer film forms coating and covering the exposed surface of the object. As the object is withdrawn, excess lacquer drains off into the floating layer leaving a coating of the lacquer upon the exposed surface of the object.
- 85 Any portions of the lacquer broken away from the floating layer during the operation tend to separate in the aqueous liquid body as globules which quickly rise and on
- 90 contact with the floating lacquer layer again to join it.
- 95 My invention will be further illustrated by the following example: A lacquer composition consisting of 150 lbs. of cellulose
- 100 nitrate, 5 gals. of tricresyl phosphate, 35 gals. of toluol, 25 gals. of ethyl acetate and 20 gals. of butyl acetate may be employed in conjunction with a liquid body of water, or better of a saturated solution of sodium
- 105 chloride or potassium iodide. The dipping operation may then be carried out as has been described in connection with the apparatus illustrated in the drawings using a lacquer and a liquid body of these compositions.
- 110 In the foregoing lacquer composition, 30 pounds of the cellulose nitrate may, for example, be replaced with 50 lbs. of ester gum, and the toluol may, for example, be replaced in part by turpentine or petroleum benzine or in whole or in part by other diluents or diluent mixtures. Likewise, solvents other than ethyl acetate and butyl acetate may be employed.
- 115 Cellulose nitrate as commercially available usually contains about 30% by weight of ethyl alcohol, the cellulose nitrate being wet with the alcohol to reduce the fire hazard, and commercial ethyl acetate and commercial butyl acetate usually contain
- 120
- 125
- 130

about 15% of ethyl alcohol and about 10% of butyl alcohol respectively. It will accordingly be apparent that, if these commercial materials in the form in which they 5 are usually available are employed in a lacquer used in carrying out an operation similar to that described in the above example, ethyl alcohol, which is soluble in water and which dissolves water, will be present in 10 substantial amounts. Where the amount of alcohol is not excessive, lacquer compositions made from the commercial materials in their usual form may nevertheless be floated on an aqueous bath, and, where an excessive 15 amount of alcohol is so introduced into the lacquer composition, satisfactory results can be secured by employing a saline liquid body of suitable composition, such as a saturated solution of sodium chloride or potassium iodide.

In some cases, when the dipping operation is continued for prolonged periods, an emulsification of the lacquer in the aqueous body or of water from the aqueous body in 25 the lacquer may tend to take place, and this is usually due either to the presence in the lacquer composition or in the aqueous body of components which tend to promote such emulsification or to the maintenance of excessive temperatures in the dipping bath. Certain gums which are sometimes employed in lacquers, for example, may tend to promote emulsification. With respect to temperature, the dipping operation is best carried out at temperatures as low as can conveniently be maintained, although refrigeration is not essential. The operation can be carried out with a lacquer composition of the type described above with bath temperatures of from 70 to 75° F. or higher although a better separation between the lacquer layer and the liquid body may be maintained by the maintenance of lower temperatures. The dipping bath may, for example, be cooled by circulating water or other cooling medium through pipe coils arranged in the dipping tank or in heat exchanging relation with the walls of the dipping tank to maintain bath temperatures of from 40 to 65° F., although lower temperatures may be used. Low bath temperatures have the further advantages of retarding evaporation from the bath and of assisting in the application of relatively thick single coats with any particular lacquer composition. If emulsification proceeds to any objectionable extent, the lacquer layer and the emulsified part of the dipping bath may be withdrawn and run through a filter or a centrifuge or otherwise treated to break the emulsion.

The lacquer coating which I obtain in carrying out my invention is of good quality, free from bloom or blush, and of improved 65 smoothness. While polishing operations

may still be desirable or necessary to produce certain types of finishes when using my invention, I have found that the amount of polishing and the intensity of the operation may be materially reduced, consequently enabling a substantial reduction in the time, labor and expense involved in the polishing operation. One or more coats may be applied according to my invention. The thickness of the individual coat can be controlled 70

by regulating the viscosity of the lacquer and the speed at which the object or objects to be dipped are immersed and withdrawn. With a straight panel, such as that illustrated in the drawing, the speed of immersion may be as much as 8" per minute or somewhat more and the speed of withdrawal may be in the neighborhood of 6" per minute or somewhat less. I find it advantageous to so regulate the speed of withdrawal that opportunity is provided for substantially all excess of lacquer to drain from the object or objects dipped as they are withdrawn and so that dipping of lacquer from the lower edges of the object or objects after they are withdrawn is substantially avoided. Other things being the same, a thicker coating is obtained as the viscosity of the lacquer composition is increased and as the speed of withdrawal is increased. 95

I have found my invention to be a particularly advantageous way of applying relatively thick lacquer coatings in a single dip. While my invention is of general utility in connection with the application of cellulose ester lacquers, in the case of pigmented lacquers containing relatively heavy pigments it is sometimes necessary to modify the operation in order to provide for sufficient separation between the floating lacquer 100 layer and the supporting liquid body in the dipping bath. With lacquer compositions containing comparatively light pigments or relatively small amounts of light pigments, such as a black lacquer pigmented with lamp black, water alone may be used as the supporting liquid body. With lacquers containing heavy pigments, however, it is sometimes advantageous to employ heavier liquid bodies, such as concentrated solutions of 105 sodium chloride or potassium iodide or of other salts which dissolve to form heavy saline solutions immiscible with the lacquer composition employed.

My invention is of particular utility in connection with the application of flat or dull finish lacquer coatings, or coatings simulating a rubbed finish. For this purpose, cellulose ester lacquers containing metallic soaps such as the stearates of zinc or aluminum, or containing finely divided gums which are insoluble or which become insoluble upon evaporation of the solvent, may be employed. Due to the improved application of the lacquer obtained in carrying out my invention, for many purposes flat finishes of satisfac- 110 115 120 125 130

tory quality can be obtained by my invention using such lacquer compositions without the necessity of any smoothing operation or with very materially reduced expenditure of time and labor in smoothing.

6. While I have described my invention particularly in connection with the use of an aqueous liquid body for floating the lacquer layer, it will be apparent that other liquid bodies of greater density than the lacquer used and which are substantially immiscible with the lacquer are useful in the application of cellulose ester lacquers in accordance with my invention.

15. My invention has several important advantages. From the standpoint of operation, it will be apparent that I have provided a method of applying cellulose ester lacquers by dipping which is applicable where a large aggregate surface is coated in a single operation and which at the same time avoids the necessity of using large volumes of the lacquer. By avoiding the use of excessively large volumes of the cellulose ester lacquer, I avoid or minimize fire hazards, I reduce the expense and I make it easier to maintain the composition of the lacquer bath. I also provide an operation in which cheap liquids may be employed for floating the lacquer layer, for example water or saline solutions such as a solution of sodium chloride may be used. From the standpoint of the lacquer coating obtained, my invention enables the production directly from the dipping operation of a coating of improved smoothness reducing the amount of smoothing or polishing necessary to secure smooth or glossy finishes. My invention also provides an operation in which bloom or blush of the lacquer coat due to the presence of water is avoided. My invention also is advantageous in the application of relatively thick individual lacquer coats.

I claim:

1. An improved method of applying cellulose ester lacquers, which comprises floating a layer of the cellulose ester lacquer on a liquid body of greater density which is substantially immiscible with the lacquer and dipping the object to which the lacquer is to be applied through the floating layer of cellulose ester lacquer.

2. An improved method of applying cellulose ester lacquers, which comprises floating a layer of the cellulose ester lacquer on

a liquid body of greater density which is 55 substantially immiscible with the lacquer, the lacquer being substantially free from components substantially soluble in the liquid body, and dipping the object to which the lacquer is to be applied through the 60 floating layer of cellulose ester lacquer.

3. An improved method of applying cellulose ester lacquers, which comprises floating a layer of cellulose ester lacquer substantially free from components substantially soluble in or capable of dissolving water on an aqueous body of greater density which is substantially immiscible with the lacquer and dipping the object to which the lacquer is to be applied through the floating 70 layer of cellulose ester lacquer.

4. An improved method of applying cellulose ester lacquers, which comprises floating a layer of the cellulose ester lacquer on a body of an aqueous saline solution of greater density which is substantially immiscible with the lacquer and dipping the object to which the lacquer is to be applied through the floating layer of cellulose ester lacquer.

5. An improved method of applying cellulose ester lacquers, which comprises floating a layer of the cellulose ester lacquer on a body of an aqueous solution of sodium chloride and dipping the object to which the lacquer is to be applied through the floating layer of lacquer.

6. An improved method of applying cellulose ester lacquers, which comprises floating a layer of cellulose ester lacquer substantially free from components substantially soluble or capable of dissolving water on a body of aqueous saline solution of greater density which is substantially immiscible with the lacquer and dipping the object to which the lacquer is to be applied through the floating layer of the cellulose ester lacquer.

7. An improved method of applying cellulose ester lacquers, which comprises floating a layer of the cellulose ester lacquer on an aqueous body of greater density which is substantially immiscible with the lacquer and dipping the object to which the lacquer is to be applied through the floating layer of cellulose ester lacquer.

In testimony whereof I affix my signature.

REME A. BEAUSEJOUR.